

July 2, 1929.

F. E. FIELD

1,718,950

TRANSMISSION SYSTEM

Filed March 31, 1926

Fig. 1



Fig. 2



Fig. 3



Fig. 4

Inventor:  
Frank E. Field

by J. S. Roberts Atty.

## UNITED STATES PATENT OFFICE.

FRANK E. FIELD, OF SOMERVILLE, NEW JERSEY, ASSIGNOR TO WESTERN ELECTRIC COMPANY, INCORPORATED, OF NEW YORK, N. Y., A CORPORATION OF NEW YORK.

## TRANSMISSION SYSTEM.

Application filed March 31, 1926. Serial No. 98,758.

This invention relates to transmission systems and particularly to transmission systems employing transformers.

An object of the invention is to improve 5 the transmission characteristics of electric circuits.

A related object of the invention is to repeat a wide range of frequencies with substantially uniform efficiency.

10 A specific object of the invention is to reduce the resonance peak in the transmission characteristic curve of an amplifying device, caused by resonance effects between the capacity existing across the terminals of the 15 amplifying device and the inductance of an input transformer.

The invention is particularly applicable to radio broadcasting, electrical phonographic recording and reproducing and similar systems in which transformers are employed to couple an incoming circuit of resistive impedance to the capacitive impedance represented, for example, by the grid-filament circuit of a space discharge tube 25 amplifier.

In systems of this type it is important that the amplifier have a substantially flat gain characteristic over a wide frequency range in order to faithfully transmit or reproduce 30 the essential music or speech frequencies. It is well known, however, that the inductance of an input transformer of an amplifier will resonate with the distributed capacity of the transformer and the capacity of the amplifier, producing a peak in the transmission 35 characteristic curve. As a result, the gain of the amplifier at and near the resonance frequency is greater than the gain at the other transmitted frequencies, and in some 40 cases may be so pronounced that the amplifier will sing or howl at the resonance frequency.

This difficulty is largely overcome, in accordance with this invention, by utilizing 45 the eddy current loss in a transformer to give the transformer a flat transmission characteristic over a wide frequency range. According to a feature of the invention, the magnetic structure of the transformer is so 50 arranged that the effective inductance of the transformer is high at very low frequencies and there is very little eddy current loss, resulting in a high gain. As the frequency

rises, however, the eddy current loss increases and the effective inductance of the transformer decreases. By thus materially decreasing the inductance of the resonant circuit at the higher frequencies, it is possible, within certain limits, to raise the resonance to such a predetermined point that it will 60 have no effect on the transmission efficiency of the transformer within the frequency range to be transmitted.

The various features and advantages of the invention will be described in detail in 65 connection with the accompanying drawing, in which:

Fig. 1 is a diagrammatic illustration of an amplifier circuit embodying the invention;

Fig. 2 is a perspective view of a transformer having a magnetic core constructed 70 in accordance with the invention;

Fig. 3 shows curves illustrating the drop in effective permeability of various thicknesses of core material with increases in frequency; and 75

Fig. 4 shows curves illustrating the characteristics of several different transformer circuits.

In Fig. 1, an incoming line 5 is connected 80 to an outgoing line 6 by means of a two-stage amplifier comprising space discharge tubes 7 and 8 connected in tandem. Direct current is supplied to the cathodes of these tubes from the battery 9, and space current is supplied to 85 the anodes from battery 10. Grid polarizing batteries 11 and 12 are associated with the tubes 7 and 8, respectively. The line 5 is coupled to the input circuit of tube 7 by means of an input transformer 13. The tubes 7 and 8 are coupled together by an interstage transformer 14, and the output circuit of the tube 8 is coupled to the outgoing line 6 by means of an output transformer 15. The 90 transformers 13, 14 and 15 comprise primary 95 and secondary windings and are designed to transmit a wide band of frequencies.

It is well known that the effective permeability of magnetic materials varies with the frequency of the magnetizing force to 100 which it is subjected. This is due to the action of the eddy currents in the material which cause a diminution of the effective flux and hence a drop in the effective permeability. According to this invention the magnetic circuits of transformers 13 and 14 are 105

so constructed that the eddy current loss is very small at low frequencies, but increases greatly in response to slight increases in the frequency of the transmitted waves. Such a transformer, as hereinafter described, may have a precomputed eddy current loss factor which will give the transformer a substantially flat transmission characteristic over the required frequency range.

The input transformers 13 and 14 may be of the type illustrated in Fig. 2. This transformer comprises two similar E-shaped magnetic core sections 26 and 27 wound in the usual manner with superimposed primary and secondary windings indicated generally at 28. Any suitable type of clamping device may be employed to hold the assembled structure intact.

A suitable magnetic material for the core sections 26 and 27 is a nickel-iron alloy known as permalloy, which, when subjected to the proper heat treatment, has an extremely high permeability when operated at low flux densities. This material is a composition consisting chiefly of nickel and iron containing from 30% to 90% nickel, depending upon the particular characteristics desired. Particularly good results have been obtained with a composition consisting of approximately 78½% nickel and 21½% iron. The characteristics and method of preparing these alloys are disclosed in a United States Patent 1,586,884 granted to G. W. Elmen, dated June 1, 1926, and are also described in some detail in a paper by H. D. Arnold and G. W. Elmen entitled "Permalloy", published in the May 1923 issue of the Journal of the Franklin Institute.

It is a property of permalloy that its permeability at very low magnetizing forces is extraordinarily high, values of the order of 6,000 for zero magnetizing force being easily obtainable, whereas the corresponding value for the best grade of iron is only about 300. The value of the permeability at zero force is obtained by determining a series of values for exceedingly low forces, say of the order of .01 gauss to .05 gauss. The results plot linearly and may be extrapolated back to the value for  $H=0$ .

The eddy current loss in permalloy core transformers increases with the frequency of the transmitted waves much more rapidly than in transformers employing other types of magnetic cores, such as iron or silicon steel. The eddy current loss, however, may be controlled by constructing the permalloy core in a plurality of sections or laminations of predetermined thickness, the several sections or laminations being insulated from each other when comparatively small eddy current losses are desired. In order to provide a core having an extremely high eddy current loss factor, the core may consist of uninsulated laminations, since the oxide coating produced

during the heat treatment of permalloy has a low resistance, or it may even consist of a solid core, depending upon the particular characteristics desired.

In describing the preferred method of designing transformers having any desired characteristics, reference is made to C. P. Steinmetz's "Theory and Calculation of Transient Electric Phenomena and Oscillations" page 359, where the following formula is given:

$$B_m = \frac{B_i}{cl_o \sqrt{2}} \sqrt{\frac{\epsilon^{+2cl_o} + \epsilon^{-2cl_o} - 2 \cos 2cl_o}{\epsilon^{+2cl_o} + \epsilon^{-2cl_o} + 2 \cos 2cl_o}}$$

in which,

$B_m$  = apparent flux density

$B_i$  = flux density produced by external magnetomotive force

$$c = \sqrt{0.4\pi^2 f^2 \lambda \mu 10^{-8}}$$

$l_o$  = ½ the thickness of the laminations

$f$  = frequency

$\mu$  = permeability at zero frequency

$\lambda$  = electrical conductivity.

This formula gives the relation between the flux density at zero frequency and any other frequency. Since the flux density is proportional to the permeability this formula can be used to determine the permeability of magnetic materials at various frequencies.

Assuming that silicon steel has a normal zero frequency permeability of 320 and a conductivity of  $2 \times 10^4$ , the permeability of 14 mil laminations at various frequencies may be computed. This data is illustrated graphically by the curve 30 of Fig. 3 in which the ordinates represent the percentage permeability and the abscissæ represent kilocycles.

The curves 31, 32, 33 and 34 illustrate the permeability at various frequencies of permalloy laminations comprising 78½% nickel and 21½% iron, which are 6 mils, 14 mils,  $\frac{1}{16}$  inch and  $\frac{1}{8}$  inch thick, respectively. The permalloy employed in all of the samples is assumed to have a zero frequency permeability of 10,000 and a conductivity of  $6.24 \times 10^4$ . It will be seen from curves 31, 32, 33 and 34 that as the thickness of the permalloy laminations is increased, the drop in permeability becomes greater, the drop in the case of permalloy laminations  $\frac{1}{8}$  inch in thickness, represented by curve 34 being about 94% at 500 cycles. These calculations are based on the assumption that the laminations are thoroughly insulated from each other, as by means of shellac. However, when no insulation is employed, the effect is the same as that of much thicker laminations, approaching that of a solid core at the higher frequencies. The effect of this drop in permeability on the characteristics of an input transformer may be illustrated in the following manner.

An input transformer may be represented

analytically by an inductance  $L$  shunted by a capacity  $C$ . The value of  $L$  is the total inductance that the transformer would have if the primary and secondary windings were connected in series. The capacity  $C$  is the total of the various small capacities in the transformer between turns, layers and sections of the windings expressed as the equivalent capacity shunted across the secondary terminals of the transformer. This parallel combination of  $L$  and  $C$  will resonate at a frequency obtained by the relation

$$2\pi f = \sqrt{\frac{1}{LC}}$$

in which  $L$  is expressed in henries,  $C$  in farads, and  $f$  in cycles per second. Knowing the inductance of a transformer and the distributed capacity of the particular type of winding used, it is possible by means of this relation to calculate the resonance frequency of the transformer. Let it be assumed, for example, that an input transformer winding of a certain type has a distributed capacity of 20 micro-microfarads, and, when a silicon steel core made up of 14 mil laminations is inserted, has a total inductance of 500 henries. The resonance frequency, calculated by means of the above formula, is approximately 1590 cycles. Curve 30 of Fig. 3 shows that at this frequency, the permeability has not begun to drop and hence the transformer will actually resonate at 1590 cycles.

When the silicon steel core is replaced with a permalloy core comprising a plurality of 14 mil laminations, the total inductance of the transformer will now be at least 5000 henries, and a calculation by means of the above formula shows that the resonance point will be at 500 cycles assuming that the permeability remains constant. Actually, however, the permeability does not remain constant since, as shown by curve 32 of Fig. 3, at 500 cycles the permeability has been reduced to 36% of its original value, or 3600, which results in an inductance at that frequency of 1800 henries. This inductance would cause resonance at 837 cycles if the permeability remained constant, but at that frequency the permeability has been reduced to 28% of its original value, resulting in an inductance of 1400 henries. This inductance would resonate with the capacity at 950 cycles were it not for the fact that at this point the permeability is still further reduced. Following this method it is found that the transformer would actually resonate at about 1,000 cycles. That is, the action of the eddy currents in the core has resulted in raising the resonance point from 500 cycles to 1,000 cycles.

Let it now be assumed that the 14 mil laminated permalloy core is replaced by a core of the same material having laminations  $1/8$  inch thick, as illustrated graphically by curve 34 of Fig. 3. By a series of calculations, it

is found that the transformer would then resonate at a frequency of about 4300 cycles. In this case the action of the eddy currents has resulted in a shift of the resonance point from 500 cycles to 4300 cycles.

In a circuit such as that illustrated in Fig. 1 when transformers of fairly high ratio are employed, the maximum amplification is obtained at the frequency at which the inductance of the transformer resonates with the effective capacity across its secondary winding. This is true, for example, when the turns ratio of the transformer is greater than 5 to 1 and when the impedance of the circuit to which the primary of the transformer is connected is more than 20,000 ohms. At frequencies above and below the resonance frequency the amplification falls off rapidly. For lower turns ratio or lower impedances in the circuit connected to the primary, the curve flattens out considerably. With a silicon steel core such as that described above the amplification characteristic will be as shown by the curve 40 of Fig. 4, in which the ordinates represent voltage amplification and the abscissæ frequency in cycles per second. When 14 mil permalloy laminations are employed the resonance point is lowered and the transmission characteristic curve is flattened out as shown by the curve 41. The lowering of the resonance point in this case is due to the much higher inductance of the windings. Curves 42 and 43 show the shape of the transmission characteristic when  $1/6$  inch and  $1/8$  inch permalloy laminations are employed, respectively, the resonance point being raised in each case because of the lowering of the inductance due to the action of the eddy currents. As the resonance point is raised, the curve becomes flatter and the quality of the transmitted speech and music is improved.

The capacity of the vacuum tube and the rest of the circuit connected directly to the secondary of the transformer has for clarity been neglected in this discussion. It will, however, add directly to the distributed capacity of the transformer and produce a corresponding lowering of the resonance frequency.

The input transformer 13 of Fig. 1, for example, when constructed in accordance with the invention has a high effective inductance and very little eddy current loss at low frequencies. As the frequency rises, however, the eddy current loss increases and the effective inductance of the transformer decreases. Since the capacity effectively in shunt to the secondary winding remains practically constant, the frequency at which the inductance of the transformer resonates with the effective shunt capacity is raised to a point where it has no effect on the transmission efficiency of the transformer within the frequency range transmitted.

The invention is, of course, susceptible of various other modifications and adaptations not specifically referred to but included within the scope of the appended claims.

5. What is claimed is:

1. A signalling system having substantially uniform transmission over a wide range of frequencies, including an inductive element the field of which contains a magnetic 10 element having an eddy current loss increasing with frequency at signaling field strengths, the eddy current loss in said element being large at frequencies at which the other parts of the system tend to introduce 15 a bend in the transmission characteristic whereby the tendency to the production of such bend in the characteristic is effectively opposed.

2. A signaling system having substantially uniform transmission over a wide range of frequencies, including an inductive element the field of which contains a magnetic element comprising an alloy consisting chiefly of nickel and iron and having an eddy 25 current loss increasing with frequency more rapidly than iron at signaling field strengths, said element being laminated, the eddy current loss in said element being large at frequencies at which the other parts of the system would introduce a bend in the transmission 30 characteristic.

3. A wave transmission system comprising two circuits across one of which an appreciable capacity effect exists, means for coupling said circuits comprising inductance which tends to resonate with said capacity, and means associated with said inductance for controlling the frequency of said resonance comprising a magnetic structure the 40 permeability of which decreases greatly in response to slight increases in the frequency of the transmitted waves.

4. A wave transmission system comprising two circuits across one of which an appreciable capacity effect exists, means for coupling said circuits comprising inductance which tends to resonate with said capacity, and means associated with said inductance for controlling the frequency of said resonance comprising a magnetic structure having a higher initial permeability than silicon steel and proportioned to cause the value of the permeability to decrease greatly in response to slight increases in the frequency of 55 the transmitted waves.

5. A wave transmission system comprising two circuits across one of which an appreciable capacity effect exists, a transformer for coupling said circuits and comprising inductance which tends to resonate with said capacity, and a magnetic structure for said transformer comprising an alloy consisting chiefly of iron and nickel having a higher permeability than silicon steel at zero frequency and proportioned to cause the value

of the permeability to decrease a predetermined percentage in response to slight increases in the frequency of the transmitted waves.

6. A wave transmission system comprising two circuits across one of which an appreciable capacity effect exists, a transformer for transmitting a band of frequencies comprised within the essential range of speech and music between said circuits, said transformer comprising inductance which tends to resonate with said capacity, and means to cause the frequency of said resonance to occur at a point near the upper limit of said band comprising a magnetic structure for said transformer which causes the value of said inductance to decrease materially in response to increases in the frequency of the transmitted waves.

7. A transmission system comprising two circuits across one of which an appreciable capacity effect exists, a transformer for transmitting a wide band of frequencies between said circuits, said transformer comprising mutual inductance which tends to resonate with said capacity, and means for varying the value of said mutual inductance within predetermined limits comprising a magnetic core for said transformer composed of a plurality of insulated laminations of a material having a higher permeability at low magnetizing forces than silicon steel, said laminations being proportioned in thickness to cause the eddy current losses in said core to vary in magnitude in response to changes in the frequency of the transmitted waves such that the resonant frequency between said capacity and said mutual inductance is raised and the effective band width of the transmission characteristic is increased.

8. A transmission system comprising two circuits across one of which an appreciable capacity effect exists, a transformer for transmitting a wide band of frequencies between said circuits, said transformer comprising mutual inductance which tends to resonate with said capacity, and means for varying the value of said inductance within predetermined limits comprising a magnetic core for said transformer composed of an alloy consisting chiefly of nickel and iron, in which the nickel content is between 35% and 90% of the whole and is so proportioned that the eddy current losses therein vary materially in magnitude in response to changes in the frequency of the transmitted waves.

9. In a transmission system comprising an incoming line and an outgoing line, a circuit for repeating from said incoming line to said outgoing line electrical variations included within a wide frequency band, said circuit having a capacity of the order of magnitude of the interelectrode capacity of a space discharge amplifier, said circuit including a transformer comprising inductance which

tends to resonate with said capacity and the distributed capacity of said transformer at a frequency in the lower region of said band, and a magnetic structure for said transformer the permeability of which decreases materially in response to increases in the frequency of said variations to raise the actual frequency of said resonance to a point well above the point attainable when the permeability of 10 said magnetic structure remains constant.

10. In a transmission system comprising an incoming line and an outgoing line, a circuit for repeating from said incoming line to said outgoing line electrical variations extending over a wide frequency band, said circuit having a capacity of the order of magnitude of the interelectrode capacity of a space discharge amplifier, said circuit including a

transformer comprising inductance which tends to resonate with said capacity and the distributed capacity of said transformer at a frequency in the lower region of said band, and a magnetic core for said transformer composed of an alloy consisting chiefly of nickel and iron in which the nickel content 20 is 78½% or thereabouts of the whole and formed of a plurality of laminations of such cross-sectional area that the permeability of said core decreases materially in response to increases in the frequency of said variations, whereby the actual frequency of said resonance is raised to a point in the neighborhood of the upper region of said band.

In witness whereof, I hereunto subscribe my name this 29 day of March, A. D. 1926.

FRANK E. FIELD.